

# UNITED STATES PATENT OFFICE.

JESSE B. BRONSTEIN AND CHARLES E. WALLER, OF ALLENTOWN, PENNSYLVANIA,  
ASSIGNORS TO TROJAN POWDER COMPANY, OF NEW YORK, N. Y., A CORPORATION  
OF NEW YORK.

## AMMONIUM-NITRATE EXPLOSIVE.

1,343,077.

Specification of Letters Patent.

Patented June 8, 1920.

No Drawing.

Application filed February 5, 1920. Serial No. 356,478.

*To all whom it may concern:*

Be it known that we, JESSE B. BRONSTEIN and CHARLES E. WALLER, citizens of the United States, and residents of Allentown, 5 Lehigh county, Pennsylvania, have invented certain Improvements in Ammonium-Nitrate Explosives, of which the following is a specification.

This invention relates to improvements in 10 explosives and more particularly to explosives containing ammonium nitrate.

In our U. S. Patent 1,188,244 we have described nitrostarch explosives, in which ammonium nitrate sensitized with T. N. T. is 15 used as a substitute for part of the nitrostarch in the explosive composition.

We have now discovered that a mixture 20 of ammonium nitrate and T. N. T. or equivalent agent, in which the T. N. T. or equivalent agent is present in amount insufficient to wholly sensitize the ammonium nitrate, is capable of detonation when admixed with a relatively small amount of a detonating agent, such as nitro starch, and that in this 25 way an explosive is obtained which has particularly desirable properties for use in coal mining and for other uses where an explosive of comparatively low shattering power, but of high moving or heaving effect is 30 desired.

An explosive made according to the present invention is particularly desirable for mining coal, since it brings down the coal in lumps of the type and size that are most 35 salable, and with a minimum production of "fines."

In forming our explosive we first prepare 40 a mixture of the ammonium nitrate and trinitrotoluene, the trinitrotoluene being either simply mixed with the ammonium nitrate, or heated to its fusion point, so as to 45 form a coating on the ammonium nitrate particles. Any equivalent agent, such as a nitro naphthalene or a nitro benzene, may be employed as the sensitizing material, in place of the trinitrotoluene; the amount, however, of the sensitizing agent employed, being insufficient to effect complete sensitization 50 of the ammonium nitrate. A mixture containing more than 90% of the ammonium nitrate, and consequently less than 10% of the sensitizing agent, has been found suited to our purpose, such mixture being substantially non-explosive, not exploding with a

detonator containing a charge of one gram 55 of mercury fulminate.

This partially sensitized but very insensitive mixture we now mix with a primary detonating agent such as nitrostarch, enough 60 of the nitrostarch or equivalent material being employed to reinforce the sensitizing agent already present with the ammonium nitrate sufficiently to render the entire mixture explosive. The nitrostarch surrounds and partly coats the incompletely sensitized 65 granules of ammonium nitrate in such a manner that the particles of nitrostarch remain substantially unmixed with the other elements, and they therefore form a substantially homogeneous ground mass capable of 70 transmitting detonation, and of assisting in detonating the partially but incompletely sensitized granules of ammonium nitrate.

Thus, as in the preferred forms of our invention, we may use ammonium nitrate 75 partially sensitized with from four to eight per cent. of trinitrotoluene or equivalent agent, and may add to from 80 to 90 parts of such partially sensitized ammonium nitrate from 20 to 10 parts of nitrostarch, or 80 equivalent thereof, together with from one-fourth of 1% to 1% of mineral oil, and from one-fourth of 1% to 1% of zinc oxid or any equivalent anti-acid material.

As a specific example of our explosive the 85 following formula is given:

|                          |        |
|--------------------------|--------|
| Nitrostarch              | 15.0%  |
| Ammonium nitrate mixture | 84.2%  |
| Zinc oxid                | .4%    |
| Mineral oil              | .4%    |
|                          | 90     |
|                          | 100.0% |

The composition of the ammonium nitrate mixture in the above formula is 93% ammonium nitrate and 7% T. N. T. 95

As a further example, and one in which a small amount of sodium nitrate is added in place of part of the ammonium nitrate mixture, the following is given: 100

|                          |        |
|--------------------------|--------|
| Nitro-starch             | 15.0%  |
| Ammonium nitrate mixture | 79.2%  |
| Sodium nitrate           | 5.0%   |
| Zinc oxid                | .4%    |
| Mineral oil              | .4%    |
|                          | 105    |
|                          | 100.0% |

The addition in the foregoing example of the sodium nitrate reduces correspondingly the amount of the ammonium nitrate mixture in the explosive, but it is not desirable to reduce the amount of partially sensitized substance below 70% of the finished explosive.

We claim:—

1. An explosive comprising a substantially non-explosive mixture of ammonium nitrate and an explosive material capable in sufficient quantity of sensitizing said nitrate, and sufficient of a detonating agent to render the entire mixture explosive.
- 10 2. An explosive comprising a substantially non-explosive mixture of ammonium nitrate and a nitro-hydrocarbon capable in sufficient quantity of sensitizing said nitrate, and sufficient of a detonating agent to render the entire mixture explosive.
- 15 3. An explosive comprising a substantially non-explosive mixture of ammonium nitrate and an explosive material capable in sufficient quantity of sensitizing said nitrate, and sufficient of a nitrated carbo-hydrate to render the entire mixture explosive.
- 20 4. An explosive comprising a substantially non-explosive mixture of ammonium nitrate and a nitro-hydrocarbon capable in sufficient quantity of sensitizing said nitrate, and sufficient of a nitrated carbohydrate to render the entire mixture explosive.
- 25 5. An explosive comprising a substantially non-explosive mixture of ammonium nitrate and trinitrotoluene, and sufficient of a detonating agent to render the mixture explosive.
- 30 6. An explosive comprising a substantially non-explosive mixture of ammonium nitrate and trinitrotoluene, and sufficient nitrostarch to render the mixture explosive.
- 35 7. An explosive comprising a substantially non-explosive mixture of ammonium nitrate and an explosive material capable in sufficient quantity of sensitizing said nitrate and sufficient nitrostarch to render the entire mixture explosive.
- 40 8. An explosive comprising a mixture of ammonium nitrate and trinitrotoluene, said trinitrotoluene forming less than 10% of said mixture, and sufficient of a detonating agent to render the mixture explosive.
- 45 9. An explosive comprising a mixture of ammonium nitrate and trinitrotoluene, said trinitrotoluene forming less than 10% of said mixture, and sufficient nitrostarch to render the mixture explosive.
- 50 10. An explosive comprising a mixture of ammonium nitrate and trinitrotoluene, said trinitrotoluene forming less than 10% of said mixture, and said mixture forming not less than 70% of the finished explosive, and sufficient of a detonating agent to render the mixture explosive.
- 55 11. An explosive comprising a mixture of

ammonium nitrate and trinitrotoluene, less than 10% of the said mixture being trinitrotoluene, and sufficient nitrostarch to render the mixture explosive, said ammonium nitrate mixture forming not less than 70% of the finished explosive.

12. An explosive comprising 70 to 90 parts of a mixture of ammonium nitrate and trinitrotoluene, said mixture containing less than 10% trinitrotoluene, and 10 to 20 parts 75 nitrostarch.

13. The process of forming an explosive which consists of preparing a substantially non-explosive mixture of ammonium nitrate and an explosive material capable in sufficient quantity of sensitizing said nitrate, and admixing with said mixture a sufficient quantity of a detonating agent to render the entire mixture explosive.

14. The process of forming an explosive 85 which consists of preparing a substantially non-explosive mixture of ammonium nitrate and trinitrotoluene, and admixing with said mixture sufficient of a detonating agent to render the entire mixture explosive.

15. The process of forming an explosive which consists of preparing a substantially non-explosive mixture of ammonium nitrate and an explosive material capable in sufficient quantity of sensitizing said nitrate and 95 admixing with said mixture a sufficient quantity of nitrostarch to render the entire mixture explosive.

16. The process of forming an explosive which consists of preparing a substantially non-explosive mixture of ammonium nitrate and trinitrotoluene, and admixing with said mixture sufficient nitrostarch to render the entire mixture explosive.

17. The method of forming an explosive 105 which consists of incompletely sensitizing ammonium nitrate with trinitrotoluene, and adding sufficient nitrostarch to completely sensitize the entire mixture.

18. The method of forming an explosive 110 which consists of incompletely sensitizing ammonium nitrate with a suitable sensitizing material, and adding sufficient of a detonating agent to completely sensitize the entire mixture.

19. The method of forming an explosive 115 which consists of coating particles of ammonium nitrate with sufficient of sensitizing material to incompletely sensitize said nitrate, and admixing with said incompletely 120 sensitized particles, sufficient of a detonating agent to completely sensitize the entire mass.

20. The method of forming an explosive 125 which consists of coating particles of ammonium nitrate with sufficient trinitrotoluene to incompletely sensitize said nitrate, and admixing with said incompletely sensitized particles sufficient of a detonating agent to completely sensitize the entire mass.

21. The method of forming an explosive which consists of coating particles of ammonium nitrate with sufficient of a sensitizing material to incompletely sensitize said nitrate, and admixing with said incompletely sensitized particles sufficient nitrostarch to completely sensitize the entire mass.

22. The method of forming an explosive which consists of coating particles of ammonium nitrate with sufficient trinitrotoluene to incompletely sensitize said nitrate, and admixing with said incompletely sensitized particles sufficient nitrostarch to completely sensitize the entire mass.

23. The process of forming an explosive which consists of preparing a substantially non-explosive mixture of ammonium nitrate and trinitrotoluene, heating said mixture to the fusion point of the trinitrotoluene, and admixing with the resulting material suffi-

cient of a detonating agent to render the entire mass explosive.

24. The process of forming an explosive which consists of preparing a substantially 25 non-explosive mixture of ammonium nitrate and a sensitizing agent, heating the said mixture to the fusion point of said sensitizing agent, and admixing with the resultant material sufficient nitrostarch to render the 30 entire mass explosive.

25. The process of forming an explosive which consists of preparing a substantially 35 non-explosive mixture of ammonium nitrate and trinitrotoluene, heating said mixture to the fusion point of the trinitrotoluene, and admixing with the resultant material sufficient nitrostarch to render the entire mass explosive.

JESSE B. BRONSTEIN.  
CHARLES E. WALLER.